

1

2,912,447

## CYCLIC DIOL DIESTER LUBRICANTS

Kent C. Brannock, Kingsport, Tenn., assignor to Eastman Kodak Company, Rochester, N.Y., a corporation of New Jersey

No Drawing. Application November 29, 1957  
Serial No. 699,530

6 Claims. (Cl. 260—410)

This invention relates to a new group of compounds which have been found to be particularly suitable for use as synthetic lubricants.

Hydrocarbon or mineral lubricating oils are widely used as lubricants, but such materials suffer from certain disadvantages which limit their use in many applications. In particular, hydrocarbon oils undergo marked viscosity changes with changes in temperature and have relatively high pour points when they have a usable viscosity at high temperatures. Hydrocarbon lubricating oils having low pour points usually contain a considerable amount of volatile material which is lost at high temperatures. Hydrocarbon lubricating oils particularly suffer where extreme conditions of temperature are encountered, such as in turbo-jet aircraft engines. High engine temperatures in turbo-jet aircraft engines are desirably employed to increase engine efficiency. In such a high temperature use, conventional hydrocarbon lubricating oils suffer thermal and oxidative breakdown to an undesirable degree.

In recent years a number of synthetic ester lubricants have been proposed to overcome some of the objections to hydrocarbon lubricating oils.

It is an object of this invention to provide a new group of synthetic ester materials that have particular utility as lubricants and which are not subject to many of the disadvantages inherent to hydrocarbon lubricating oils.

It is another object of the invention to provide novel synthetic ester lubricants which have lower pour points than hydrocarbon lubricants of comparable viscosity.

It is another object of this invention to provide a new class of synthetic ester lubricants having improved resistance to thermal degradation.

It is likewise an object of this invention to provide new synthetic ester lubricants especially adapted to meet the high temperature requirements desired for lubricating turbo-jet engines and for related uses.

Other objects will be apparent from the description and claims which follow.

The class of compounds embodying the invention are diesters of cyclic diols selected from the group consisting of compounds having the formulas:



and

2



5

- 10 Wherein R is an alkyl group containing 6 to 11 carbon atoms. Typical cyclic diesters of the invention include: 1,1-cyclopentanedimethanol di-n-heptanoate; 1,1-cyclopentanedimethanol di-n-octanoate; 1,1-cyclopentanedimethanol dipelargonate; 1,1-cyclopentanedimethanol di-n-decanoate; 1,1-cyclopentanedimethanol di-n-undecanoate; 1,1-cyclopentanedimethanol di-n-dodecanoate; 1,1-cyclohexanhexanedimethanol di-n-heptanoate; 1,1-cyclohexanhexanedimethanol di-n-octanoate; 1,1-cyclohexanhexanedimethanol di-n-decanoate; 1,1-cyclohexanhexanedimethanol di-n-dodecanoate; 2,2-norcamphenedimethanol di-n-heptanoate; 2,2-norcamphenedimethanol di-n-octanoate; 2,2-norcamphenedimethanol dipelargonate; 2,2-norcamphenedimethanol di-n-decanoate; 2,2-norcamphenedimethanol di-n-undecanoate and 2,2-norcamphenedimethanol di-n-dodecanoate.

The present synthetic diesters of cyclic diols have considerable utility as lubricants. By varying the choice of the acyl moiety with which the 1,1-cyclopentanedimethanol; 1,1-cyclohexanhexanedimethanol and 2,2-norcamphenedimethanol are esterified, lubricants having a wide range of viscosities and pour points can be obtained. The present diesters can be used directly as lubricants or they can be blended with other lubricants. If desired, minor proportionate amounts of such conventional lubricant additives as antioxidants, extreme pressure additives, viscosity index improvers, thickeners, anticorrosion agents and related materials can be incorporated into the present diester lubricants.

The viscosity and pour point characteristics of typical synthetic diesters of cyclic diols embodying this invention are illustrated in Table 1 below. In addition, a comparison is made with a typical hydrocarbon oil of comparable viscosity.

40

TABLE 1

| 60 | Lubricant                                     | Kinematic Viscosity<br>in Centistokes |         | Pour<br>Point,<br>°F. |
|----|-----------------------------------------------|---------------------------------------|---------|-----------------------|
|    |                                               | 100° F.                               | 210° F. |                       |
|    | Typical hydrocarbon oil                       | 13.0                                  | 2.6     | -30                   |
|    | 1,1-Cyclopentanedimethanol di-n-octanoate     | 9.70                                  | 2.65    | <-75                  |
| 55 | 1,1-Cyclopentanedimethanol dipelargonate      | 12.03                                 | 3.02    | -60                   |
|    | 1,1-Cyclohexanhexanedimethanol di-n-octanoate | 13.32                                 | 3.12    | -65                   |
|    | 2,2-Norcamphenedimethanol di-n-octanoate      | 17.18                                 | 3.57    | <-65                  |

60

As can be seen from the data set out in Table 1, the present synthetic lubricants have excellent viscosity and pour point characteristics.

65

The improved thermal stability of the present synthetic diester lubricants is illustrated by the data in Table 2 and Table 3 below. For purposes of comparison, two known diester lubricants, namely, bis-(2-ethylhexyl)-sebacate and 2,2,4-trimethyl-1,3-pentanediol dipelargonate, as well as an 8 carbon branched chain oxo alcohol diester of cyclohexane-1,1-diacetic acid, are compared with typical diesters of the present invention by the data in Table 2 and Table 3.

3  
TABLE 2

| Ester                                                        | Percent change in<br>100° F. viscosity<br>after 8 hour heating<br>at indicated tempera-<br>ture |
|--------------------------------------------------------------|-------------------------------------------------------------------------------------------------|
| Bis-(2-ethylhexyl) sebacate                                  | -18% at 600° F.                                                                                 |
| 2,2,4-Trimethyl-1,3-pentanediol dipelargonate                | -16% at 550° F.                                                                                 |
| 3 Carbon oxo alcohol diester of 1,1-cyclohexanediacetic acid | -19% at 600° F.                                                                                 |
| 1,1-Cyclopentanedimethanol dipelargonate                     | -1.4% at 600° F.                                                                                |
| 1,1-Cyclohexanedimethanol di-n-octanoate                     | +0.6% at 600° F.                                                                                |
| 2,2-Norcamphanedimethanol di-n-octanoate                     | +2.9% at 600° F.                                                                                |

TABLE 3

| Ester                                                        | Percent Decomposition/hour at— |         |         |         |         |
|--------------------------------------------------------------|--------------------------------|---------|---------|---------|---------|
|                                                              | 500° F.                        | 525° F. | 550° F. | 575° F. | 600° F. |
| Bis-(2-ethylhexyl) sebacate                                  | 0.03                           | 0.11    | 0.13    | 0.59    | 1.3     |
| 2,2,4-Trimethyl-1,3-pentanediol dipelargonate                | 0.1                            | —       | 1.09    | —       | —       |
| 3 Carbon oxo alcohol diester of 1,1-cyclohexanediacetic acid | 0.04                           | —       | 0.17    | —       | 1.6     |
| 1,1-Cyclopentanedimethanol dipelargonate                     | —                              | 0.02    | 0.03    | —       | 0.04    |
| 1,1-Cyclohexanedimethanol di-n-octanoate                     | —                              | —       | —       | 0.003   | 0.01    |
| 2,2-Norcamphanedimethanol di-n-octanoate                     | —                              | —       | —       | 0.01    | 0.05    |

The data in Table 2 and Table 3 point-up the fact that the synthetic lubricants of the present invention can be utilized at high temperatures as they possess excellent resistance to thermal degradation.

The pour point data set out in Table 1 was determined by ASTM Method D-97-47 and the viscosity data set out in Table 1 and Table 2 was determined by ASTM Method D-88-44. The data set out in Table 3 concerning the percent decomposition/hour of the various esters was based on the determination of the acid produced on heating samples of the various esters under nitrogen for eight hour periods.

The following examples illustrate the preparation of typical diesters of the present invention from starting materials known in the art.

*Example 1*

A mixture of 147 g. of cyclopentanecarboxaldehyde, 331 g. of 36% formalin and sufficient methanol to make a homogeneous solution, was added dropwise to a stirred solution of 105 g. of potassium hydroxide in 375 ml. of methanol over a 40 minute period. The resulting mixture was then heated under reflux for 5½ hours, cooled, and 400 ml. of water added. The mixture was thereafter distilled until removal of the methanol was complete, and on cooling the residue, 1,1-cyclopentanedimethanol crystallized out. The 1,1-cyclopentanedimethanol crystals were removed from the reaction mixture by filtration, washed in cold water, and recrystallized from a hexane-chloroform mixture to give 123 g. of 1,1-cyclopentanedimethanol having a melting point of 98.5-99.5° C. Thereafter, 1,1-cyclopentanedimethanol so prepared was esterified to prepare the present diester lubricants.

(a) A mixture of 156 g. (1.2 moles) of 1,1-cyclopentanedimethanol, 346 g. (2.4 moles) of n-octanoic acid and 50 ml. of xylene was refluxed in a reactor fitted with a Dean-Stark separator until water ceased to be evolved from the reaction mixture. The theoretical amount of water, 43 ml., was collected after 3 hours and the temperature of the reaction mixture had risen to 272° C. The resulting mixture was cooled, and thereafter washed with 100 ml. of a 5% sodium hydroxide aqueous solution and then with 100 ml. of water. The xylene was stripped off by distillation and the resulting distillation residue further distilled in a molecular still to give 1,1-cyclopentanedimethanol di-n-octanoate boiling at 97-

101° C. at 10 microns of mercury and having  $n_D^{20}$  1.4559.

(b) In lieu of n-octanoic acid in the process described above, 2.4 moles of pelargonic acid and 1.2 moles of 1,1-cyclopentanedimethanol were reacted to prepare 1,1-cyclopentanedimethanol dipelargonate boiling at 107-110° C. at 6 microns of mercury and having  $n_D^{20}$  1.4575.

*Example 2*

10 A mixture of 1.2 moles of 1,1-cyclohexanedimethanol and 2.4 moles of n-octanoic acid was reacted and worked-up as described in Example 1 (a) above. The 1,1-cyclohexanedimethanol di-n-octanoate prepared boiled at 115-120° C. at 5.4 microns of mercury and had  $n_D^{20}$  1.4601.

*Example 3*

A 137 g. sample of bicyclo(2,2,1)-5-heptene-2,2-dimethanol was hydrogenated over 15 g. of Raney nickel at 100° C. under a pressure of 1,000 p.s.i. to give 2,2-norcamphanedimethanol. A mixture of 1.2 moles of 2,2-norcamphanedimethanol and 2.4 moles of n-octanoic acid was reacted and worked-up as described in Example 1 (a) above. The 2,2-norcamphanedimethanol dicaprate prepared boiled at 130-136° C. at 1 micron of mercury and had  $n_D^{20}$  1.4670.

While the above examples describe the esterification of 1,1-cyclopentanedimethanol; 1,1-cyclohexanedimethanol and 2,2-norcamphanedimethanol with particular organic acids, it is to be understood that in a like manner these cyclic diols can be esterified with any organic acid having the formula



wherein R is an alkyl group containing 6 to 11 carbon atoms. Likewise, mixtures of such acids can be utilized to prepare the present diester lubricants.

Thus, by means of this invention, a novel and highly useful group of synthetic diester lubricants is provided. The improved physical characteristics make the present diesters eminently suitable for use as lubricants in applications where hydrocarbon lubricating oils are now used, as well as in high temperature applications where hydrocarbon lubricating oils are completely unsuitable. Because of their improved thermal stability at high temperatures, the present diester lubricants have particular utility for use in turbo-jet aircraft engines and for related high temperature applications.

The invention has been described in considerable detail with particular reference to certain preferred embodiments thereof, but it will be understood that variations and modifications can be effected within the spirit and scope of the invention as described hereinabove and as defined in the appended claims.

55 I claim:

1. A synthetic lubricant composition of high thermal stability consisting essentially of a diester selected from the group consisting of compounds of the formula:



65 and



70 wherein R is an alkyl group containing 6 to 11 carbon atoms.

5

2. A synthetic lubricant composition of high thermal stability consisting essentially of a diester of the formula:



wherein R is an alkyl group containing 6 to 11 carbon atoms. 10

3. A synthetic lubricant composition of high thermal stability consisting essentially of a diester of the formula:



wherein R is an alkyl group containing 6 to 11 carbon atoms. 20

6

4. A synthetic lubricant composition of high thermal stability consisting essentially of 1,1-cyclopentanedimethanol di-n-octanoate.

5. A synthetic lubricant composition of high thermal stability consisting essentially of 1,1-cyclopentanedimethanol dipelargonate.

6. A synthetic lubricant composition of high thermal stability consisting essentially of 2,2-norcamphanedimethanol di-n-octanoate.

References Cited in the file of this patent

UNITED STATES PATENTS

|              |                     |               |
|--------------|---------------------|---------------|
| 2,738,370    | Staib et al. -----  | Mar. 13, 1956 |
| 15 2,817,673 | Roelen et al. ----- | Dec. 24, 1957 |

FOREIGN PATENTS

|              |                     |               |
|--------------|---------------------|---------------|
| 569,404      | Great Britain ----- | May 23, 1945  |
| 20 1,087,168 | France -----        | Feb. 22, 1955 |